

Dec. 3, 1957

W. BETTERIDGE ET AL  
NICKEL CHROMIUM ALLOY AND ELECTRICAL RESISTANCE  
HEATING ELEMENTS MADE THEREOF  
Filed July 14, 1953

2,815,283



INVENTORS  
WALTER BETTERIDGE  
HARRY LEWIS

BY C. Dr. Dreher  
ATTORNEY

## 1

2,815,283

## NICKEL CHROMIUM ALLOY AND ELECTRICAL RESISTANCE HEATING ELEMENTS MADE THEREOF

Walter Betteridge, Solihull, and Harry Lewis, Kings Heath, Birmingham, England, assignors to The International Nickel Company, Inc., New York, N. Y., a corporation of Delaware

Application July 14, 1953, Serial No. 367,852

Claims priority, application Great Britain July 17, 1952

## 2 Claims. (Cl. 75—171)

The present invention relates to a special nickel-chromium heat resistant alloy and, more particularly, to electrical resistance heating elements made of such alloys and having improved service life when subjected in use to elevated temperatures, especially under conditions involving repeated heating and cooling.

It is known that nickel-chromium alloys used for electrical resistance heating elements may advantageously contain small amounts of both calcium and cerium (or other rare earth metal) for the purpose of increasing the service life, and that these alloys may contain small amounts of other elements, e. g., silicon. In making the alloys, the cerium is commonly used as Mischmetall, and the term "cerium" is used herein to mean not only cerium itself but also any other rare earth metals present. In practice the silicon contents of nickel-chromium alloys containing both calcium and cerium have hitherto been very low, e. g., of the order of 0.5%. While such nickel-chromium alloys have been found beneficial when employed as electrical resistance heating elements, demands by industry for heating elements with greatly improved service lives have placed further burdens on such alloys with the result that the problem of providing improved alloys to meet the needs of industry has been greatly accentuated. Although many attempts were made to meet the needs and demands of industry, none, as far as applicants are aware, were entirely successful when carried into practice commercially on an industrial scale.

We have discovered that by employing a higher and critical silicon content in conjunction with a very low and critical cerium content, it is possible very considerably to increase the service life of an electrical resistance element made of such an alloy. To be forgeable, the alloy must also contain a small and critical amount of calcium.

It is an object of the present invention to provide a special heat resistant nickel-chromium alloy having improved service life at elevated temperatures.

It is another object of the present invention to provide special electrical resistance heating elements characterized by improved performance at elevated service temperatures, especially under conditions involving repeated heating and cooling.

Other objects and advantages will become apparent from the following description taken in conjunction with the accompanying drawing in which:

Figure 1 is a curve showing the critical effect of silicon on the average life in hours of a nickel-chromium alloy containing a critical amount of cerium and tested in accordance with designation B 76-39 of the American Society for Testing Materials (ASTM); and

Figure 2 depicts a curve showing the critical effect of cerium on the average life in hours of a nickel-chromium alloy containing a critical amount of silicon likewise tested in accordance with the aforementioned ASTM designation B 76-39.

According to the invention, nickel-chromium alloys for

## 2

electrical resistance heating elements contain from 10 to 25% chromium, from 0.005 to 0.05% calcium, 0.01 to 0.1% cerium and 1.15 to 2% silicon, the balance (except for impurities) being nickel. Preferably the elements are present in narrower ranges, namely from 15 to 25% chromium, from 0.01 to 0.03% calcium, from 0.025 to 0.06% cerium and from 1.4 to 1.6% silicon.

Although the invention is concerned with nickel-chromium alloys, as distinguished from nickel-chromium-iron alloys, iron is often present as an impurity in the raw materials and in consequence the alloys of the invention may contain up to 2% iron. Moreover, some of the nickel (in an amount up to 15% of the total alloy) may be replaced by cobalt.

The alloys may contain various other elements without detriment, namely up to 1% aluminum, up to 0.3% carbon, up to 0.16% copper and up to 3% manganese. The impurities present may include traces of various elements, e. g., titanium.

In evaluating heat resistant alloys of the type containing 80% nickel and 20% chromium for use as electrical resistance heating elements, an accelerated life test is employed in accordance with the American Society for Testing Materials designation B 76-39. In this test, the alloy specimen in the form of a wire measuring about 12 inches long and having a diameter corresponding to not larger than No. 20 American Wire Gauge (A. W. G.) nor smaller than No. 22 A. W. G. (i. e., within the range of about 0.025 inch to 0.032 inch) is subjected to intermittent heating and cooling under prescribed conditions at a temperature of about 2150° F. (1177° C.), the heating being accomplished by passing electric current through the wire. The service lives of electrical resistance wires of a number of alloys have been measured in accordance with the aforementioned ASTM test. The percentage compositions of some of the alloys tested and the results obtained are given in the following table:

Table

| Alloy No. | Percent Ca | Percent Ce | Percent Si | Percent Al | Percent Cr | Percent Fe | Life, hours |
|-----------|------------|------------|------------|------------|------------|------------|-------------|
| 1-----    | 0.015      | 0.08       | 0.55       | 0.17       | 20.8       | 0.39       | 145         |
| 2-----    | 0.010      | 0.05       | 1.37       | 0.28       | 20.4       | 0.45       | 444         |
| 3-----    | 0.010      | 0.03       | 1.47       | 0.42       | 19.8       | 0.34       | 490         |

The first alloy (No. 1) was a typical alloy as marketed hitherto. The second alloy (No. 2) had a silicon content which, though much higher than usual hitherto, was still below the preferred range of the present invention. The third alloy (No. 3) has silicon and cerium contents both within the preferred ranges. The results of tests conducted on the alloy provided by the invention indicated that markedly improved service lives are obtained when the alloy contains about 0.03% to 0.05% cerium, particularly when the alloy contains 1.4% to 1.6% silicon.

The way in which the service life varies with the silicon content is illustrated by Figure 1 of the accompanying drawings, which is a graph showing the average lives obtained with electrical resistance wires of alloys containing about 0.010% calcium, 0.04% cerium, 0.2% aluminum, 20% chromium and 0.4% iron and of varying silicon contents. It will be seen that as the silicon content rises above the normal low figure, there is no appreciable increase in the service life until it is about 1.0%. At this figure the service life begins to increase at a rate which itself rapidly increases. Between 1.15 and 1.4%, the increase is most striking, the service life rising to at least three times the value at 0.6% silicon. When the silicon content exceeds 1.4%, the life remains approximately constant up to 2%.

The critical nature of the cerium content is illustrated

by Figure 2 of the accompanying drawings, which is a graph showing the average lives obtained with electrical resistance wires of alloys containing about 0.010% calcium, 0.2% aluminum, 1.5% silicon, 20% chromium and 0.4% iron, and of varying cerium contents. It will be seen that in the narrow range of 0.03 to 0.05% cerium, the best lives are obtained. Generally, alloys provided by the invention exhibit service lives at 2150° F. (1177° C.) as determined by the ASTM designation B 76-39 of the order of about 400 hours and higher, while the best commercially available alloys of the 80-20 nickel-chromium type of which we are aware do not show good lives of this order when tested in this manner.

The term service life in this specification refers in all cases to the total life to burn-out of the wire, since this occurs before the resistance of the wire has increased by 10 percent.

Although the present invention has been described in conjunction with preferred embodiments, it is to be understood that modifications and variations may be resorted to without departing from the spirit and scope of the invention, as those skilled in the art will readily understand. Such modifications and variations are considered to be within the purview and scope of the invention and appended claims.

We claim:

1. An electric resistance heating element made of a nickel-chromium alloy consisting essentially of 15% to 25% chromium, 0.01% to 0.03% calcium, 1.4% to 1.6% silicon, 0.03% to 0.05% cerium, up to 15% cobalt, up to 2% iron, up to 3% manganese, up to 1%

aluminum, up to 0.16% copper, up to 0.3% carbon, and the balance consisting essentially of nickel, said electric resistance heating element being characterized by markedly improved service life of at least 400 hours when subjected to intermittent heating and cooling at an elevated temperature of 2150° F. in accordance with ASTM designation B 76-39.

2. A heat resistant nickel-chromium alloy adapted for the manufacture of electrical resistance heating elements and consisting essentially of 15% to 25% chromium, 0.01% to 0.03% calcium, 1.4% to 1.6% silicon, 0.03% to 0.05% cerium, up to 15% cobalt, up to 2% iron, up to 3% manganese, up to 1% aluminum, up to 0.16% copper, up to 0.3% carbon, and the balance consisting essentially of nickel, said alloy being characterized by improved service life of at least 400 hours when subjected as an electrical resistance wire to intermittent heating and cooling at an elevated temperature of 2150° F. in accordance with ASTM designation B 76-39.

20

References Cited in the file of this patent

UNITED STATES PATENTS

|           |        |       |               |
|-----------|--------|-------|---------------|
| 1,465,547 | Driver | ----- | Aug. 21, 1923 |
| 2,174,919 | Kay    | ----- | Oct. 3, 1939  |
| 2,581,420 | Lohr   | ----- | Jan. 8, 1952  |

OTHER REFERENCES

Ser. No. 124,858, Hessenbruch (A. P. C.), published June 1, 1943.